

## UNITED STATES PATENT OFFICE

2,327,127

STAIN AND CORROSION RESISTANT TIN  
SURFACE AND METHOD OF PRODUCING  
THE SAME

Frank E. Rath, Bellevue, Pa.

No Drawing. Application February 26, 1940,  
Serial No. 320,967

9 Claims. (Cl. 148—6)

This invention relates to the treatment of surfaces of tin or tin alloys in order to make them stain and corrosion resistant. More particularly it relates to the treatment of the surfaces of tin plate or tin plate containers to render them stain and corrosion resistant without materially affecting their appearance.

Tin, in general, may be regarded as a corrosion resistant metal and, as such, has found widespread application in the arts as a protective coating for steel and other metals. Tin coated steel is universally accepted as the most suitable material for the manufacture of containers for food and many other products. However, a tinned surface is subject to a number of defects since tin is not absolutely inert but will react to a limited extent with certain types of materials. These reactions are not particularly serious in themselves but insofar as many of them result in discoloration of either the tin surface or the food product packed in the container, they are objectionable. Some typical examples of reactions of this sort and the defects resulting therefrom are:

(1) Oxidation of tin plate during storage or in the baking operation during enameling or lacquering, this resulting in a type of discoloration known as "yellow stain." This stain is generally regarded as an interference film of tin oxide. Electrodeposited tin plate produced commercially is especially subject to this type of discoloration.

(2) Discoloration of the exterior of tin cans during the retort processing of food products, this being usually a purplish stain and may be classed as steam oxidation. It seldom occurs if the air is completely swept out of the retort.

(3) Discoloration of the interior of tin cans by foods such as corn, peas, beans, corned beef, sea foods and many other products which contain sulphur bearing protein matter, reactions of this type resulting in purple or black sulphide areas on the tin plate. With some foods, such as corn, small particles of the food itself are darkened.

(4) Etching of the tin by corrosive food such as pumpkin, spinach, hominy, sweet potatoes, or acid fruits, in some cases etching being accompanied by discoloration. In many foods etching is not very severe and hence is not troublesome. Where etching is severe, however, it is objectionable from an appearance standpoint and for other reasons.

(5) Decoloration or bleaching of fruits and vegetables by reaction between the coloring matter of the fruit and the tin, this being especially true of red fruits.

(6) Reaction between beer and metallic tin, this resulting in turbidity of the beer and a deterioration of the flavor.

Defects of type 3, 4, 5 and 6 and others of a

similar nature have resulted in the widespread practice of enameling the interior of tin cans for many uses. Although enameling has been fairly effective in combating these defects, it is expensive and in the case of corrosive fruits there is always the possibility of a break in the enamel coat with the result that corrosion will be concentrated on that spot and perforation of the can may occur. Further, most enamels require baking at elevated temperatures (400°-425° Fahrenheit) and during this process "yellow staining" of the tin plate is apt to occur. Enameling is not effective in preventing oxidation of the tin surface, as evidenced by the fact that "yellow stain" will form beneath the enamel during baking.

Attempts have been made to prevent dark sulphide stains by methods other than enameling. Schutte, in the United States Patent, No. 2,624,951, discloses the prevention of sulphide discolorations by oxidizing the surfaces of tin containers by means of a permanganate solution. This method, while successful, is subject to a number of limitations. Cook and Romine, in United States patent application Serial No. 270,913, discloses the use of electrochemical anodic oxidation as a more satisfactory means for producing the same result. Although these processes are more or less successful in preventing sulphide discoloration of tin by nearly neutral foods, they are ineffective in preventing etching by foods of a more corrosive nature.

From the foregoing, it is apparent that no general method exists for treating tin surfaces to eliminate all the previously described defects. The practice of enameling is the closest approach to such a general method, and is practical in only a limited number of cases and will not prevent "yellow stain."

Generally stated, the present invention consists in treating tin plate, tin or tin alloy surfaces with an acid solution containing phosphate ions. The appearance of the tin surface is not changed by the treatment but the treated surfaces are readily distinguished by their resistance to oxidation, resistance to attack by dilute acids and resistance to staining by food products, especially those foods which contain sulphur compounds. Since tin and tin oxides are known to react with phosphoric acid to produce highly insoluble and relatively inert compounds, I believe it is not unreasonable to assume that as a result of the treatment the tin surface is provided with a dense superficial protective film of an insoluble phosphate compound which is a substantially integral part of said surface. Such a protective film would function as a barrier preventing contact of the tin and substance with which tin normally reacts and thus would prevent the reactions previously mentioned.

Since the appearance of the treated tin surface is not changed, the film is superficial in nature. This lack of thickness prevents its positive identification by ordinary chemical means. However, the conditions for the effective treatment of the tin surface are those most favorable to the formation of stannic oxyphosphate. I believe, therefore, that the film formed is this compound, which is sometimes referred to simply as stannic phosphate.

The evidence leading to the above conclusion is:

1. A tin surface which carries or is provided with a film of oxide can be effectively treated in a hot acidified solution of a soluble phosphate compound, whereas the treatment of a "chemically clean" tin surface in such a solution is relatively ineffective. I believe this difference is due to the fact that phosphoric acid reacts with stannic oxide to produce stannic oxyphosphate while the reaction of this acid with metallic tin produces a stannous phosphate.

2. A chemically clean tin surface can be effectively treated if an oxidizing agent is added to the treating solution. The presence of the oxidizing agent demands the formation of a stannic compound. The only readily formed quadravalent tin compound of phosphoric acid, known to me, is stannic oxyphosphate.

3. The treatment of a "chemically clean" tin surface with a solution containing an oxidizing agent is more effective than the treatment of an "oxidized" tin surface. In the latter case the conditions are such that a stannous phosphate as well as stannic phosphate could be formed, hence I conclude that conditions favorable to the formation of a film consisting substantially of stannic oxyphosphate, are to be preferred.

As indicated in the above discussion of the nature of the protective film, two methods may be practiced under the present invention. The first and simpler method requires the presence of an oxide film on the surface to be treated. Pretreatment of the surface in the first method is not involved, however, since sufficient oxide film is present on all tin surfaces, even immediately after manufacture, to meet this requirement. The product of the first method is a tin surface which will not "yellow stain" and is more resistant to other types of defects than are ordinary tin surfaces but the treated surface cannot be said to be substantially free from the latter. The product of the simplified treatment is applicable only where freedom from "yellow stain" is the important characteristic and the conditions of service with regard to defects of other types are not severe.

In practicing the present invention in its simplest form the tin surface is immersed for a period of 5-10 seconds in a hot (200°-212° Fahrenheit) solution containing phosphate anions and alkali metal cations, for example of the following composition:

|                                               |                   |
|-----------------------------------------------|-------------------|
| Di-sodium phosphate, $Na_2HPO_4 \cdot 12H_2O$ | 100 gms./liter    |
| Ortho-phosphoric acid, $H_3PO_4$ (85%)        | 25 ml./liter      |
| Water                                         | To make one liter |

The above composition provides a solution with a pH of about 3.0. On removal from the solution the tin surface is rinsed and dried in any convenient manner. A lubricant may be applied to the treated surface, if desired, to

facilitate handling in subsequent manufacturing steps.

In addition to the ingredients already mentioned, it has been found desirable to add a small quantity of a wetting agent to reduce the surface tension of the treating solution. The wetting agent promotes immediate contact of the tinned surface and the solution, thus facilitating the film formation. Any wetting agent which is stable in an acid solution may be used. An example of a wetting agent which has been used successfully is "Duponol 80," a compound currently marketed under this name by E. I. du Pont de Nemours & Company.

15 While in the example cited above, di-sodium phosphate is the main ingredient of the treating solution, I do not wish to be limited to its use. This material is chosen as preferable because it is readily soluble and is a cheap source of phosphate ion. The sodium ion does not enter into the reactions which take place at the tin surface. Other soluble phosphate compounds could be substituted without affecting the ultimate result.

20 25 Regarding acidity of the treating solution, I have observed that the effectiveness of the treatment increases as the solution is made more acid. The increase is marked over the pH range of 6.8 (minimum acidity) to 3.5. Reducing the pH below 2.5, however, has but very slight benefit and may increase the tendency for etching of the tin to occur. For the best results compatible with economic operation, I recommend a pH range of 3.5 to 2.5.

30 35 In adjusting the acidity of the solution, I have specified the use of ortho-phosphoric acid,  $H_3PO_4$ . Other acids, however, may be used for this purpose. Ortho-phosphoric acid was chosen as it permits easy regulation of the pH within the 40 range 3.5 to 2.5 and also contributes to the phosphate content of the solution.

45 50 As to operating temperature of the solution, I have observed that the efficiency of the treatment improves with increasing temperature; also, that the time required for treatment decreases as the temperature of the solution is increased. Hence, in practice, I prefer to operate the solution as hot as possible, namely, at or near the boiling point of the solution.

55 60 Concentration limitations of the treating solution are discussed below:

1. Di-sodium phosphate,  $Na_2HPO_4 \cdot 12H_2O$ ; the concentration of this ingredient may be varied over a range of 25 to 200 grams per liter. Less than 25 grams per liter is insufficient for acceptable results. The effectiveness of the treatment improves as the concentration of this material is increased. The improvement between 100 and 200 grams per liter, however, is slight, and increasing the concentration beyond 200 grams per liter is therefore uneconomical.

65 70 2. Ortho-phosphoric acid,  $H_3PO_4$ : The amount required depends on the pH desired as well as the concentration of di-sodium phosphate used. If it is desired to operate within the recommended pH range (3.5 to 2.5), the amount of acid required varies directly with the di-sodium phosphate content in the approximate ratio of 1 ml. of  $H_3PO_4$  (85%) to 4 grams of  $Na_2HPO_4 \cdot 12H_2O$ .

75 70 3. "Duponol 80" (wetting agent): Use, optional; amount, not critical—2.5 ml. per liter is sufficient.

The first method treatment outlined above is designed primarily to produce a tin surface which

will not "yellow stain." While the product of this treatment is also more resistant than ordinary tin surfaces to defects of other types, where substantially complete elimination of defects, i. e., "dark sulphide stains," etching, etc., as well as "yellow stain," is necessary, the second method of treatment should be used.

This second method requires that the tin surface be chemically clean before immersion in the acidified phosphate solution, and this solution must contain an oxidizing agent. A very uniform protective film of substantially pure stannic phosphate is formed under these conditions.

Any method of obtaining a chemically clean surface may be used in preparing the tin for treatment. I prefer, however, a cathodic cleaning step. In such a step the electro-chemical reactions taking place at the cathode surface reduce and remove any oxide or other chemical compound present while the action of the solution, aided by the hydrogen evolution, removes all grease, oil, dirt, etc. While any electro-cleaning solution may be used, I recommend an acid solution of similar composition to the treating solution. This is particularly desirable in a commercial unit as it eliminates elaborate rinsing equipment otherwise necessary to prevent contamination of the treating solution by dragout from the cleaning equipment.

The composition of the preferred cleaning solution is:

|                                                                           |                |
|---------------------------------------------------------------------------|----------------|
| Di-sodium phosphate, $\text{Na}_2\text{HPO}_4 \cdot 12\text{H}_2\text{O}$ | 100 gms./liter |
| Ortho-phosphoric acid, $\text{H}_3\text{PO}_4$ (85%)                      | 7 ml./liter    |
| Anhydrous chromic acid, $\text{CrO}_3$                                    | 2.5 gms./liter |

Operating conditions of the cleaning solution are:

1. The pH of this solution is about 6.2. A more acid solution may be used. However, I have found that the best results are obtained in the pH range of 6.8 to 8.0.

2. The solution is preferably operated at room temperature.

3. Any current density between 25 and 100 amperes per square foot may be used.

4. A time of treatment of 3 to 5 seconds is sufficient under most conditions.

5. The  $\text{Na}_2\text{HPO}_4 \cdot 12\text{H}_2\text{O}$  content may be varied from 25 to 200 grams per liter.

6. The quantity of  $\text{H}_3\text{PO}_4$  used depends on the pH desired and the concentration of  $\text{Na}_2\text{HPO}_4 \cdot 12\text{H}_2\text{O}$ . Other acids may be substituted for this constituent. For example, it may be found desirable to use acetic acid,  $\text{CH}_3\text{COOH}$  since this acid permits ready adjustment of the pH within the range 6.8 to 8.0.

In using a cathodic cleaning step I have observed that improved results in the subsequent treating procedure are obtained if:

1. Following the electro-cleaning operation the tin surface is allowed to stand in the cleaning solution with current off for 5-10 seconds.

On completion of this pre-treatment the tin plate is removed from the above solution and immersed for a period of 3 seconds in a hot (200°-212° Fahrenheit) solution of the following composition:

|                                                      |                |
|------------------------------------------------------|----------------|
| $\text{Na}_2\text{HPO}_4 \cdot 12\text{H}_2\text{O}$ | 100 gms./liter |
| $\text{H}_3\text{PO}_4$ (85%)                        | 25 ml./liter   |
| $\text{CrO}_3$                                       | 2.5 gms./liter |
| Duponol 80                                           | 2.5 ml./liter  |

The tin plate is then thoroughly rinsed, dried

and, if desired, a lubricant is applied to its surface to minimize scratching during subsequent handling or forming operations. The type of lubricant and method of application are entirely optional.

The product of the above treatment is a new article of manufacture, namely, a tin surface provided with a superficial film of substantially pure stannic phosphate which is characterized by substantially complete freedom from the formation of "yellow stain," "dark sulphide stain," etching by food products, etc.

In carrying out the immersion step in the second method, limitations as to solution concentration, acidity, etc., are the same as in the first method with the exception that the presence of an oxidizing agent in the treating solution for the second method is mandatory. As regards the temperature of treatment for the second method, I have noted that while the efficiency of treatment increases with temperature when treating hot dipped tin plate or tin surfaces possessing similar characteristics, making it desirable in such cases to operate at or near the boiling point of the solution; when treating electrode-deposited tin coatings, I have found that owing to the fine grain size and therefore relatively high activity of such surfaces, the treatment is best effected at considerably lower temperatures, preferably room temperature.

It is to be understood that the term "chemically clean" as used herein means that the surface is free from grease, oil and oxide films such as are normally present as a result of ordinary tin plate manufacturing methods now in current use.

I claim:

1. A new article of manufacture comprising a surface consisting essentially of metallic tin, and a protective coating on the tin, the said coating being an invisible film consisting of substantially pure stannic oxyphosphate.

2. A method of treating a tin surface to render the same substantially chemically inert, which comprises making the surface chemically clean and producing on the chemically clean surface a protective invisible film consisting of substantially pure stannic oxyphosphate by simply immersing the said surface in an aqueous solution consisting of a sodium phosphate, ortho-phosphoric acid and chromic acid.

3. A method of treating a tin surface bearing an oxide film to render the said surface substantially resistant to "yellow stain" by producing a protective phosphate film thereon, which consists in simply immersing the said surface in an aqueous solution of an alkali ortho-phosphate and phosphoric acid maintained at a pH value of from approximately 3.5 to approximately 2.5.

4. A method of treating a tin surface to render it substantially chemically inert, which comprises converting the said surface into a chemically clean condition and thereafter simply immersing it for approximately 3 seconds in a water solution consisting of essentially a sodium phosphate and chromic oxide together with sufficient ortho-phosphoric acid to slightly acidify the said solution.

5. An article having a tin surface provided with an adherent, invisible film coating consisting essentially of substantially pure stannic oxyphosphate.

6. A method of treating a tin surface to protect the same from staining, which comprises simply immersing the surface in a slightly acid

aqueous ortho-phosphate containing solution in the presence of an oxidizing agent, and producing by the simple immersion an invisible stannic oxyphosphate film on the surface.

7. A method of treating a tin surface to render the same chemically inert, which comprises making the surface chemically clean and producing on the chemically clean surface a protective, invisible film consisting of substantially pure stannic oxyphosphate by simply immersing the said surface in an aqueous solution containing a sodium phosphate, orthophosphoric acid and chromic oxide.

8. A container having a surface of metallic tin and a protective coating on the tin surface, the coating being an invisible film consisting essentially of pure stannic oxyphosphate.

9. A tin plate stock adapted to be fabricated into containers and having a protective coating on the tin plate which coating is an invisible film consisting of pure stannic oxyphosphate, produced by simply immersing the said tin plate stock in an aqueous solution containing a sodium phosphate, orthophosphoric acid, and chromic oxide.

FRANK E. RATH.